

July 9, 1946.

F. J. BOUCHARD ET AL

2,403,493

MANUFACTURING NITROCELLULOSE

Filed May 19, 1943



INVENTORS

Frederick J. Bouchard  
Robert C. Guinness  
Raphael L. Stern

BY

Cleveland B. Hellebaugh  
ATTORNEY

## UNITED STATES PATENT OFFICE

2,403,493

## MANUFACTURING NITROCELLULOSE

Frederick J. Bouchard, Radford, Va., Robert C. Gunness, Chicago, Ill., and Raphael L. Stern, South River, N. J., assignors to Hercules Powder Company, Wilmington, Del., a corporation of Delaware

Application May 19, 1943, Serial No. 487,558

12 Claims. (Cl. 260—220)

1

This invention relates to the manufacture of nitrocellulose and more particularly it relates to the recovery of spent nitrating acid adhering to nitrocellulose after separation of the nitrocellulose from the major portion of the spent acid formed in the nitration step.

Nitrocellulose is prepared by nitrating cellulose in a large excess such as 30-65 times by weight of the cellulose of "mixed acid." "Mixed acid" is a mixture of nitric acid, sulphuric acid and a relatively small proportion of water. The spent acid from the nitration is slightly weakened in nitric acid and slightly increased in water content. It is absolutely essential that it be recovered for fortification and re-use. The major part of the spent acid is relatively easily separated from the nitrocellulose. However, it is quite difficult to recover the remaining portion wetting the nitrocellulose without damaging the quality of the nitrocellulose.

It has been proposed to wash nitrocellulose containing strong spent acid with progressively more dilute spent acid so as to lose a minimum of nitric acid. This method has the serious objection that the nitrocellulose is subjected to de-nitrating conditions and becomes nonuniform and variable in ultimate degree of nitration. It has also been proposed to use wash water repeatedly until its acid concentration permitted treatment with ferrous sulphate or like reducing agent to recover nitric oxide. This method has the objection of nonuniform treatment of succeeding batches of nitrocellulose, is inefficient in nitric acid recovery, and loses sulphuric acid present. These and other methods for recovery of spent acid have either subjected the nitrocellulose to varying periods of treatment with acid or to varying concentrations causing serious nonuniformity.

Thus, in practical operation, nitrated cellulose has been removed from supernatant acid by centrifuging, squeezing or the like, to obtain nitrocellulose wet with one to three times its weight of adhering spent acid. This material has then been drowned in a large volume of water to decrease the concentration of the acid in contact with the nitrocellulose to below 2 or 3% very rapidly to prevent denitration by intermediate strength acid. The retained or adhering spent acid has been lost and has caused disposal difficulties since it has been diluted too greatly for recovery.

The process according to this invention is concerned with the recovery of the spent acid adhering to nitrocellulose after its separation from

2

supernatant spent acid. In accordance with this invention, nitrocellulose wet with such adhering spent acid is drowned by admixture with a quenching or drowning volume of an aqueous mixed acid (nitric and sulphuric acids), having a concentration between about 10% and about 25%, the volume thereof being sufficient to reduce the concentration of the resulting acid in and on the nitrocellulose from above about 75% to between about 10% and about 25% substantially instantaneously. The nitrocellulose is then removed from the drowning acid and spent acid remaining therein may be displaced, or otherwise removed by water or other washing liquid essentially water, or both. The dilute acid formed by such washing may be added to the drowning acid to permit and to aid in maintaining the concentration in the 10 to about 25% range. Nitric acid is evaporated from a portion of the drowning acid to recover a nitric acid fraction. A sulphuric acid fraction may be recovered from the evaporation residuum.

It has been found that the drowning acid of 10-25% concentration unexpectedly has substantially no denitrating effect, i. e., denitration is negligible in the period of a few minutes or few hours between drowning and complete separation of the drowning acid. At the same time it has been found practical to recover the nitric acid and sulphuric acid from the drowning acid by evaporative fractionation.

The process in accordance with this invention may be more completely described in connection with the accompanying drawing which illustrates the process diagrammatically.

Referring to the drawing the flow of pertinent material is shown as originating in a nitrator 1 from which the nitration mixture passes to a separator 2, which may be a centrifuge, squeezer, roll equipment or the like, and which removes the greater part of the spent acid from the nitrated cellulose. The free spent acid so obtained is led to storage for fortification and re-use. The nitrocellulose with adhering spent acid passes to the drowning equipment 3 where it is rapidly mixed with a large volume of drowning liquor, which reduces the concentration of the acid wetting the nitrocellulose substantially instantaneously to below denitrating levels. The nitrocellulose and drowning acids pass to a rotary filter 4 which separates the nitrocellulose from the drowning acid. Portions of drowning acid remaining in the nitrocellulose after the initial separation are washed with water, or with vapor condensate, which is essentially water, or preferably, first with the

vapor condensate and then further with water, the vapor condensate being obtained as herein-after described. The vapor condensate and/or water form a dilute acid in the washing operation, which dilute acid is admixed with separated drowning acid. The drowning acid flows from the filter back to the drowning equipment either directly or, preferably, through sedimentation equipment or a filter to remove nitrocellulose fines. The washed nitrocellulose passes from the filter into a slurry tank 5 in which it is suspended in water for subsequent purification usually in a series of tubs represented as purification equipment 6.

A portion of the drowning acid separated from the nitrocellulose, preferably a quantity about equivalent to that added in the nitrocellulose and wash liquid, is bled off and passed to a concentrator which consists of a concentration column 8 and an operatively associated evaporator 9 equipped with a suitable heating coil. The concentrator separates the drowning acid portion into the vapor fraction, essentially water vapor with a small content of nitric acid, and a liquid fraction of mixed acid of increased concentration. This mixed acid passes to an evaporator 10 equipped with a suitable heating coil. The major portion of the nitric acid in the mixed acid is evaporated from the drowning acid portion in this evaporator to form a vapor fraction containing nitric acid and water. The liquid residuum leaving the evaporator is a partially concentrated sulphuric acid fraction containing a small amount of nitric acid. This liquid passes to a sulphuric acid denitrator 13 where, by the action of steam, remaining nitric acid is evaporated to form an aqueous nitric acid vapor. The sulphuric acid liquid fraction leaves in a denitrated form. The aqueous nitric acid vapor leaving the evaporator 10 and the nitric acid vapor leaving the denitrator 13 pass with partial or no condensation to a nitric acid concentrator which consists of the concentrator column 11 and an operatively associated evaporator 12 provided with a suitable heating coil. The nitric acid concentrator resolves the nitric acid fractions fed thereto into a liquid concentrated nitric acid fraction and a vapor fraction consisting essentially of water vapor but in most cases containing a small amount of nitric acid. The vapors from one or both of the concentrators 8 and 11 may be led to a condenser 14 where they form a vapor condensate containing a small amount of nitric acid. This condensate, preferably cooled, may then be used in washing nitrocellulose on the rotary filter 4, thereby permitting complete recovery of the drowning acid from the nitrocellulose and recovery of the small amount of nitric acid in the vapor condensate. The columns 8 and 11 may be of packed or bubble-cap construction.

In a typical operation serving as an example of the process, cellulose is nitrated with 45 times its weight of mixed acid to form a spent mixed acid containing about 25% nitric acid, about 55% sulphuric acid and about 20% water. The nitration mixture is centrifuged, eliminating the major portion of the spent acid, but leaving a quantity in the nitrocellulose of about 1.1 times the weight of the nitrocellulose. The wet nitrocellulose is then drowned with mixed acid diluted to 20% total acid concentration in a quantity of approximately 50 times the weight of the nitrocellulose (dry basis). The increase in concentration in the drowning acid produced by the strong acid wetting nitrocellulose is about 2%.

The nitrocellulose is removed from the drowning acid by a rotary filter, washed on the filter by displacement first with a water vapor condensate containing about 1% nitric acid and then by a small amount of pure water. It is then treated in the usual manner for stabilization, viscosity adjustment and dehydration. The drowning acid is recycled through a sedimentation tank removing most of any associated nitrocellulose fibers. A portion of the drowning acid, substantially equivalent to the quantity added by the strong acid wetting the nitrocellulose and the wash water, is withdrawn and initially concentrated to about 45% total acid concentration. It is then evaporated to strip it of nearly all of its nitric acid to form a nitric acid water vapor fraction equivalent to about 30% nitric acid and a liquid residual fraction of about 65% sulphuric acid. The sulphuric acid is denitrated to free it of residual nitric acid by steam to yield a 65-68% sulphuric acid. The nitric acid vapors are concentrated to form a concentrated nitric acid of 66-67% nitric acid content and a vapor essentially water but containing about 1% of nitric acid. The vapors from the concentrators are condensed, cooled and used as nitrocellulose wash water to recover the nitric acid content of the drowned filtered nitrocellulose and to aid in maintaining the concentration of the drowning acid in the range desired.

It will be appreciated that it is not essential to use vapor condensate for washing the nitrocellulose. However, such operation permits substantial recovery of the small nitric acid content of the vapor condensate and it further provides a means of maintaining the drowning acid in the 10-25% range in which it is effective in drowning the nitrocellulose and at the same time recoverable. The vapor condensate in general will include nitric acid in any quantity up to about 3%. It will be appreciated that the vapor condensate may be returned directly to the drowning acid without use for washing.

Under most conditions of operation, it is necessary to add small quantities of water to the system to prevent the drowning acid from building up in concentration to a level at which denitration of nitrocellulose after drowning ceases to be negligible. Such make-up water is conveniently added by using pure water as a final wash for the nitrocellulose on the filter and merging the resultant wash water with the drowning acid. By this expedient, substantially all of the drowning acid is removed and recovered from the nitrocellulose.

The nitric acid may be recovered by distillation from the 10-25% mixed drowning acid and subsequently further concentrated. However, it has been found that preconcentration to form a mixed acid of about 35% to about 60% concentration greatly improves the efficiency of the steps of evaporating or distilling the nitric acid and subsequently concentrating it. Such preconcentration also makes practicable subsequent denitration of the residual sulphuric acid. The concentration is accomplished by evaporation of essentially water from the acid.

Usually the aqueous nitric acid fraction obtained is concentrated to 60-68%. The fraction may first be condensed but preferably the vaporous fraction with partial or no condensation is introduced directly into a concentrating column. The sulphuric acid fraction is conveniently brought to 50-75% as denitrated and may then be further concentrated in other equipment when

stronger acid is desired. The denitration step separates the small residual quantity of nitric acid, which is less than 5% of the residual fraction, from the sulphuric acid to permit ready concentration of the sulphuric acid.

It is essential that the concentration of the drowning acid be held within the range hereinabove specified. The concentration must be no greater than about 25% since otherwise denitration of the nitrocellulose occurs during and after drowning in a variable and unpredictable manner. At below concentrations of 25% and with use of the drowning acid in a volume to insure that the mixture resulting is below about 25%, substantially no denitration occurs and furthermore, the nitrocellulose obtained is highly uniform from batch to batch. Concentrations of drowning acid below about 10% do not permit obtaining the economies of the present invention since recovery of the component nitric and sulphuric acids from the acid is impractical. A concentration between 15% and 20% is preferred.

The mixed acid wetting the nitrocellulose after its removal from the major portion of the spent acid will have a total acid concentration in excess of about 75%. The ratio of sulphuric acid to nitric acid will be between about 4:1 and about 0.5:1, usually between 3:1 and 1:1, by weight. The same relationship between sulphuric acid and nitric acid will apply in the drowning acid.

The effectiveness of the present process in economic recovery of spent acid is in no small part dependent upon recovery of the drowning acid wetting the drowned nitrocellulose by means of the rotary filter which provides a filter surface through which the drowning acid may be drained, and which further provides for efficient displacement of residual acid through the filter surface with the essentially pure water of the condensed vapor obtained from the acid concentrators and with the final wash of pure water. The filter further provides a very convenient manner for introducing an amount of water to the drowning acid sufficient or nearly sufficient to maintain the concentration of the drowning acid in the critical range by compensating for the effect of the addition of strong acid in the nitrocellulose. However, it will be appreciated that water added as such or in the form of dilute acid will be in a quantity no more than that quantity which is required to maintain the concentration at the desired level in the critical range.

By maintenance of the drowning acid substantially constant in concentration, a highly uniform nitrocellulose product is obtained. It has been found that the method of this invention produces a uniform nitrocellulose of a quality fully equivalent to material obtained by drowning as heretofore with water involving complete loss of retained acid.

The present process is of particular usefulness in permitting direct and simple recovery of the nitric acid contained in the retained spent acid, and furthermore it leads to recovery of both the nitric acid and the sulphuric acid therein. In addition, the problem of disposal of waste dilute acid is avoided.

All acid concentrations herein and in the claims are in percent by weight.

What we claim and desire to protect by Letters Patent is:

1. In a procedure for manufacturing nitrocellulose in which cellulose is nitrated in an excess of mixed acid and the resulting nitrocellu-

lose is separated from supernatant spent mixed acid of above about 75% total acid concentration by weight, drowned to reduce the concentration of acid wetting the nitrocellulose rapidly to below concentrations causing substantial denitration, and then purified, a process which comprises carrying out the drowning of the said separated nitrocellulose wet with spent acid by mixing it with a quenching volume of aqueous mixed nitric and sulphuric acid having a concentration of about 10 to about 25% by weight of total acid, said volume being sufficient to reduce the concentration of the spent acid on and in the nitrocellulose to between about 10% and about 25% substantially instantaneously, removing the drowned nitrocellulose from the drowning acid, and evaporating nitric acid from a portion of the drowning acid.

2. In a procedure for manufacturing nitrocellulose in which cellulose is nitrated in an excess of mixed acid and the resulting nitrocellulose is separated from supernatant spent mixed acid of above about 75% total acid concentration by weight, drowned to reduce the concentration of acid wetting the nitrocellulose rapidly to below concentrations causing substantial denitration, and then purified, a process which comprises carrying out the drowning of the said separated nitrocellulose wet with spent acid by mixing it with a quenching volume of aqueous mixed nitric and sulphuric acid having a concentration of about 10 to about 25% by weight of total acid, said volume being sufficient to reduce the concentration of the spent acid on and in the nitrocellulose to between about 10% and about 25% substantially instantaneously, removing the drowned nitrocellulose from the drowning acid, washing the nitrocellulose with essentially water thereby obtaining a dilute acid, adding said dilute acid to the drowning mixed acid in a quantity no more than that maintaining the drowning acid between about 10% and about 25% in total acid concentration, and evaporating nitric acid from a portion of the drowning acid.

3. In a procedure for manufacturing nitrocellulose in which cellulose is nitrated in an excess of mixed acid and the resulting nitrocellulose is separated from supernatant spent mixed acid of above about 75% total acid concentration by weight, drowned to reduce the concentration of acid wetting the nitrocellulose rapidly to below concentrations causing substantial denitration, and then purified, a process which comprises carrying out the drowning of the said separated nitrocellulose wet with spent acid by mixing it with a quenching volume of aqueous mixed nitric and sulphuric acid having a concentration of about 10 to about 25% by weight of total acid, said volume being sufficient to reduce the concentration of the spent acid on and in the nitrocellulose to between about 10% and about 25% substantially instantaneously, removing the drowned nitrocellulose from the drowning acid, washing the nitrocellulose with a condensed vapor essentially water thereby obtaining a dilute acid, adding said dilute acid to the drowning mixed acid, evaporating a portion of the drowning acid to form an evaporated nitric acid fraction and a fraction of essentially water vapor, and condensing the water vapor fraction to form the aforesaid condensed vapor.

4. In a procedure for manufacturing nitrocellulose in which cellulose is nitrated in an excess of mixed acid and the resulting nitrocellulose is separated from supernatant spent mixed

acid of above about 75% total acid concentration by weight, drowned to reduce the concentration of acid wetting the nitrocellulose rapidly to below concentrations causing substantial denitration, and then purified, a process which comprises carrying out the drowning of the said separated nitrocellulose wet with spent acid by mixing it with a quenching volume of aqueous mixed nitric and sulphuric acid having a concentration of about 10 to about 25% by weight of total acid, said volume being sufficient to reduce the concentration of the spent acid on and in the nitrocellulose to between about 10% and about 25% substantially instantaneously, removing the drowned nitrocellulose from the drowning acid, evaporating a portion of the drowning acid to form a fraction of essentially water vapor, condensing the vapor fraction, and returning condensed vapor to the drowning acid in an amount permitting the concentration of the drowning acid to be maintained between about 10% and about 25% by weight.

5. In a procedure for manufacturing nitrocellulose in which cellulose is nitrated in an excess of mixed acid and the resulting nitrocellulose is separated from supernatant spent mixed acid of above about 75% total acid concentration by weight, drowned to reduce the concentration of acid wetting the nitrocellulose rapidly to below concentrations causing substantial denitration, and then purified, a process which comprises carrying out the drowning of the said separated nitrocellulose wet with spent acid by mixing it with a quenching volume of aqueous mixed nitric and sulphuric acid having a concentration of about 10 to about 25% by weight of total acid, said volume being sufficient to reduce the concentration of the spent acid on and in the nitrocellulose to between about 10% and about 25% substantially instantaneously, removing the drowned nitrocellulose from the drowning acid, evaporating a portion of the drowning acid to form a nitric acid fraction, concentrating the nitric acid fraction to form a concentrated acid fraction and a fraction essentially water vapor, condensing the said water vapor fraction, and returning the resulting condensate to the drowning acid in an amount permitting the concentration of the drowning acid to be maintained between about 10% and about 25% by weight.

6. In a procedure for manufacturing nitrocellulose in which cellulose is nitrated in an excess of mixed acid and the resulting nitrocellulose is separated from supernatant spent mixed acid of above about 75% total acid concentration by weight, drowned to reduce the concentration of acid wetting the nitrocellulose rapidly to below concentrations causing substantial denitration, and then purified, a process which comprises carrying out the drowning of the said separated nitrocellulose wet with spent acid by mixing it with a quenching volume of aqueous mixed nitric and sulphuric acid having a concentration of about 10 to about 25% by weight of total acid, said volume being sufficient to reduce the concentration of the spent acid on and in the nitrocellulose to between about 10% and about 25% substantially instantaneously, removing the drowning acid from the nitrocellulose fibers by drainage through a filter surface and by displacement of residual acid from the nitrocellulose through the filter surface with essentially water, and evaporating nitric acid from a portion of the drowning acid.

7. In a procedure for manufacturing nitrocellulose in which cellulose is nitrated in an excess

10

15

20

30

35

40

50

60

70

75

of mixed acid and the resulting nitrocellulose is separated from supernatant spent mixed acid of above about 75% total acid concentration by weight, drowned to reduce the concentration of acid wetting the nitrocellulose rapidly to below concentrations causing substantial denitration, and then purified, a process which comprises carrying out the drowning of the said separated nitrocellulose wet with spent acid by mixing it with a quenching volume of aqueous mixed nitric and sulphuric acid having a concentration of about 10 to about 25% by weight of total acid, said volume being sufficient to reduce the concentration of the spent acid on and in the nitrocellulose to between about 10% and about 25% substantially instantaneously, removing the drowned nitrocellulose from the drowning acid, evaporating nitric acid from a portion of the drowning acid, and recovering a sulphuric acid fraction of increased concentration from the said portion.

8. In a procedure for manufacturing nitrocellulose in which cellulose is nitrated in an excess of mixed acid and the resulting nitrocellulose is separated from supernatant spent mixed acid of above about 75% total acid concentration by weight, drowned to reduce the concentration of acid wetting the nitrocellulose rapidly to below concentrations causing substantial denitration, and then purified, a process which comprises carrying out the drowning of the said separated nitrocellulose wet with spent acid by mixing it with a quenching volume of aqueous mixed nitric and sulphuric acid having a concentration of about 10 to about 25% by weight of total acid, said volume being sufficient to reduce the concentration of the spent acid on and in the nitrocellulose to between about 10% and about 25% substantially instantaneously, removing the drowned nitrocellulose from the drowning acid, concentrating a portion of the drowning acid, and evaporating nitric acid from the concentrated portion to recover a nitric acid fraction and a sulphuric acid residual fraction.

9. In a procedure for manufacturing nitrocellulose in which cellulose is nitrated in an excess of mixed acid and the resulting nitrocellulose is separated from supernatant spent mixed acid of above about 75% total acid concentration by weight, drowned to reduce the concentration of acid wetting the nitrocellulose rapidly to below concentrations causing substantial denitration, and then purified, a process which comprises carrying out the drowning of the said separated nitrocellulose wet with spent acid by mixing it with a quenching volume of aqueous mixed nitric and sulphuric acid having a concentration of about 10 to about 25% by weight of total acid, said volume being sufficient to reduce the concentration of the spent acid on and in the nitrocellulose to between about 10% and about 25% substantially instantaneously, removing the drowned nitrocellulose from the drowning acid, concentrating a portion of the drowning acid, and evaporating nitric acid from the concentrated portion to recover a nitric acid fraction and a sulphuric acid residual fraction and concentrating the nitric acid fraction to 60-69%.

10. In a procedure for manufacturing nitrocellulose in which cellulose is nitrated in an excess of mixed acid and the resulting nitrocellulose is separated from supernatant spent mixed acid of above about 75% total acid concentration by weight, drowned to reduce the concentration of acid wetting the nitrocellulose rapidly to below concentrations causing substantial denitration,

and then purified, a process which comprises carrying out the drowning of the said separated nitrocellulose wet with spent acid by mixing it with a quenching volume of aqueous mixed nitric and sulphuric acid having a concentration of about 10 to about 25% by weight of total acid, said volume being sufficient to reduce the concentration of the spent acid on and in the nitrocellulose to between about 10% and about 25% substantially instantaneously, removing the drowned nitrocellulose from the drowning acid, concentrating a portion of the drowning acid, subjecting the resulting acid to evaporation to form a vapor fraction of water and a major portion of the nitric acid in the drowning acid concentrate and a liquid fraction of aqueous sulphuric acid containing the remaining nitric acid, denitrating the sulphuric acid fraction to form an aqueous nitric acid vapor, and subjecting the two said nitric vapors to concentration to form and recover a concentrated nitric acid fraction.

11. In a procedure for manufacturing nitrocellulose in which cellulose is nitrated in an excess of mixed acid and the resulting nitrocellulose is separated from supernatant spent mixed acid of above about 75% total acid concentration by weight, drowned to reduce the concentration of acid wetting the nitrocellulose rapidly to below concentrations causing substantial denitration, and then purified, a process which comprises carrying out the drowning of the said separated nitrocellulose wet with spent acid by mixing it with a quenching volume of aqueous mixed nitric and sulphuric acid having a concentration of about 10 to about 25% by weight of total acid, said volume being sufficient to reduce the concentration of the spent acid on and in the nitrocellulose to between about 10% and about 25% substantially instantaneously, removing the drowned nitrocellulose from the drowning acid, concentrating a portion of the drowning acid to form an acid concentrate fraction and a vapor fraction essentially water vapor with a small content of nitric acid, subjecting the acid concentrate to evaporation to form an aqueous nitric acid vapor fraction and a residual fraction containing the sulphuric acid of the drowning acid portion

treated, concentrating the nitric acid fraction to form a concentrated nitric acid fraction and a second vapor fraction essentially water vapor with a small content of nitric acid, condensing the two essentially water vapor fractions, and returning the condensate to the drowning mixed acid in an amount permitting the total acid concentration of the drowning acid to be maintained between about 10% and about 25%.

12. In a procedure for manufacturing nitrocellulose in which cellulose is nitrated in an excess of mixed acid and the resulting nitrocellulose is separated from supernatant spent mixed acid of above about 75% total acid concentration by weight, drowned to reduce the concentration of acid wetting the nitrocellulose rapidly to below concentrations causing substantial denitration, and then purified, a process which comprises carrying out the drowning of the said separated nitrocellulose wet with spent acid by mixing it with a quenching volume of aqueous mixed nitric and sulphuric acid having a concentration of about 10 to about 25% by weight of total acid, said volume being sufficient to reduce the concentration of the spent acid on and in the nitrocellulose to between about 10% and about 25% substantially instantaneously, removing the drowned nitrocellulose from the drowning acid, concentrating a portion of the drowning acid to form an acid concentrate fraction and a vapor fraction essentially water vapor with a small content of nitric acid, subjecting the acid concentrate to evaporation to form an aqueous nitric acid vapor fraction and a residual fraction containing the sulphuric acid of the drowning acid portion treated, concentrating the nitric acid fraction to form a concentrated nitric acid fraction and a second vapor fraction essentially water vapor with a small content of nitric acid, condensing the two essentially water vapor fractions, washing nitrocellulose wet with residual drowning acid to remove said residual acid and to form therewith a diluted acid, and adding said diluted acid to the drowning acid.

FREDERICK J. BOUCHARD.  
ROBERT C. GUNNESS.  
RAPHAEL L. STERN.